

# United States Patent Office

2,791,560

Patented May 7, 1957

1

2,791,560

## LUBRICATING GREASE THICKENED WITH A SODIUM OR LITHIUM SOAP AND INDIGO

John P. Dilworth, Fishkill, and James R. Roach, Beacon, N. Y., assignors to The Texas Company, New York, N. Y., a corporation of Delaware

No Drawing. Application April 14, 1954,  
Serial No. 423,240

12 Claims. (Cl. 252—42.1)

This invention relates to lubricating greases wherein indigo and a soap are employed in combination as thickening agents.

We have found that very superior lubricating greases are obtained by employing indigo in finely divided form as a thickening agent in conjunction with certain fatty acid soaps. The greases thus produced are characterized by very outstanding high temperature performance properties, which are generally far superior to those obtainable by employing other finely divided solid thickening agents of the prior art either as the sole thickening agent or in combination with fatty acid soaps.

The lubricating greases of our invention comprise an oleaginous liquid lubricating base thickened to a grease consistency with at least a substantial proportion of indigo in finely divided form, suitably in the form of particles not more than about one micron in diameter, and at least a substantial proportion of a sodium or lithium soap of a relatively low molecular weight soap-forming fatty acid. The composition may suitably comprise about 5 to 20 percent by weight based on the weight of the composition of indigo in finely divided form and about 5 to 20 percent by weight based on the weight of the composition of a soap of the above type, the two materials being present in amounts sufficient to thicken the composition to a grease consistency by their combined effect. The indigo and soap are preferably employed in a proportion of from about 2 to 1 to about 1 to 2 by weight.

The soaps which may be employed in these compositions are sodium and lithium soaps of fatty acids having about 12 to 16 carbon atoms per molecule, such as for example sodium laurate, lithium laurate, sodium myristate, lithium myristate, sodium palmitate, etc., as well as mixtures of such low molecular weight fatty acid soaps. The preferred soaps of this character are sodium and lithium soaps of low molecular weight fatty acids containing at least a predominant proportion of myristic acid. Also, it is to be understood that the sodium and lithium soaps are not regarded as entirely equivalent for this purpose, and in general the sodium soaps are preferred. However, both the sodium and lithium soaps of the low molecular weight fatty acids, and particularly those of myristic acid, produce a very pronounced synergistic effect in combination with indigo upon the high temperature performance properties of the grease, and are therefore both included in the purview of this invention.

The lubricating oil base may be any suitable oil of mineral, vegetable, animal or synthetic origin, such as have been employed heretofore in lubricating greases. With particular advantage, where a wide temperature range grease is desired, the oil base may comprise at least a substantial proportion of a high molecular weight polyester of lubricating characteristics.

Additives of the usual types may be employed, such as oxidation inhibitors, corrosion inhibitors, tackiness agents, extreme pressure agents, and so forth. An oxida-

2

tion inhibitor is preferably employed, which may suitably be an inhibitor of the amine type, such as diphenylamine, a-naphthylamine, b-naphthylamine, p-phenylene diamine and N,N' diphenyl p-phenylene diamine. A compound of this type may be present in amounts of from about 0.05 percent to about 5 percent by weight based on the weight of the composition. Also, additional thickening agents may be present in minor amounts, such as other soaps and other finely divided solids.

10 The preparation of these greases may be carried out by any convenient method, such as by adding the soap and the indigo either separately or together during the grease making process, or by separately forming a grease containing a sodium or lithium soap of a low molecular weight fatty acid as the chief thickening agent and a grease containing indigo in finely divided form as the chief thickening agent and then mixing the two. The soap is preferably prepared by saponifying a mixture of low molecular weight fatty acids comprising at least 20 70 percent, and preferably at least 90 percent of myristic acid and the glycerides of such acids with an aqueous solution of sodium or lithium hydroxide in the presence of a small amount of mineral lubricating oil. A small excess of sodium hydroxide may be employed in this 25 saponification; for example, the finished grease may contain about 0.02-0.2 percent of free alkali (calculated as sodium or lithium hydroxide). However, this is not an essential condition, and the grease may be neutral or even slightly acid if desired.

30 As a preferred embodiment of this invention, lubricating greases of outstandingly superior properties over a wide temperature range are obtained by employing both indigo in finely divided form and a sodium or lithium soap of a low molecular weight fatty acid as described 35 above as thickening agents in a high molecular weight polyester of the type disclosed by R. T. Sanderson in U. S. 2,628,974, obtained by reacting a dibasic aliphatic acid with a glycol and end blocking the reaction product with a monohydric aliphatic alcohol or a monocarboxylic 40 aliphatic acid. Particularly suitable polyesters of this character are products obtained by reacting a mono- or poly-alkylene glycol with a dicarboxylic acid and a monohydric alcohol, represented by the formula

R<sub>2</sub>—OOC—R<sub>1</sub>—COO—(R—OOC—R<sub>1</sub>—COO)<sub>x</sub>—R<sub>2</sub>  
45 where R is an aliphatic group or an aliphatic ether group containing from 4 to 12 carbon atoms, R<sub>1</sub> is an aliphatic group containing from 1 to 12 carbon atoms, R<sub>2</sub> is an aliphatic group containing from 1 to 12 carbon atoms, and x is an integer from 1 to 5. Preferably, R is 50 an aliphatic group or an aliphatic ether group containing from 6 to 12 carbon atoms in branched chain arrangement, R<sub>1</sub> is an alkylene group containing 7 to 8 carbon atoms, R<sub>2</sub> is an alkyl group containing from 4 to 9 carbon atoms in branched chain arrangement and x is 1 or 2. 55 An ester of this type preferably comprises from about 20 percent up to 100 percent of the oil component of the grease, the remainder being a mineral oil or other oil of a different type. The composition preferably contains 60 also about 0.1-8 percent by weight of N,N' diphenyl para-phenylene diamine and about 0.5-15 percent by weight of tricresyl phosphate.

Greases of the above type, wherein both indigo and a sodium or lithium soap of low molecular weight fatty acids are employed as thickening agents in a high molecular weight polyester, have very exceptional high temperature properties, required for the long-time lubrication of bearings at temperatures as high as 400° F., in addition to excellent low temperature properties down to -60° F.

65 The following examples are given in order to more fully disclose the invention. Example I is illustrative of attempts to obtain high temperature greases employing

indigo as the sole thickening agent. Examples 2 and 3 are illustrative of the preferred embodiment of this invention wherein both a soap of the type described above and indigo are employed as thickening agents in combination with a high molecular weight polyester of the preferred type and a particularly advantageous inhibitor combination, and Example 4 is illustrative of greases of this invention prepared from a different synthetic ester base.

## EXAMPLE 1

A grease was prepared having the following composition by weight:

|                             | Percent |
|-----------------------------|---------|
| Indigo                      | 35.0    |
| Diphenyl-p-phenylenediamine | 1.0     |
| Tricresyl phosphate         | 3.0     |
| Mineral oil                 | 4.3     |
| Synthetic ester             | 56.7    |

The synthetic ester was obtained by reacting together sebacic acid, 2-ethylhexane-1,3-diol and 2-ethylhexanol in about a 2:1:2 ratio, respectively, and consisted predominantly of the compound (iso-C<sub>9</sub>H<sub>17</sub>)<sub>2</sub>OOC-(CH<sub>2</sub>)<sub>8</sub>-COO-iso-C<sub>8</sub>H<sub>16</sub>-OOC-(CH<sub>2</sub>)<sub>8</sub>-COO-(iso-C<sub>9</sub>H<sub>17</sub>).

The mineral oil was a refined paraffinic distillate oil having an SUS viscosity at 100° F. of 330.

The indigo was the dye grade product obtained from National Aniline Division of Allied Chemical and Dye Corporation. This was in the form of a powder having an average particle size of about 0.1 micron diameter, and a measured surface area of about 10 to 50 square meters per gram.

The grease was prepared by mixing the indigo and the oleaginous base together by means of an electric stirrer until a smooth paste was formed. The inhibitors were then added and the grease was finished by milling with two passes through a Premier Colloid Mill at 0.002 and 0.0015 inch clearance.

A soft purple grease was obtained having a dropping point of 500+° F. and an ASTM worked penetration at 77° F. of 371.

## EXAMPLE 2

A grease was prepared having the following composition by weight:

|                             | Percent |
|-----------------------------|---------|
| Indigo                      | 10.0    |
| Sodium myristate            | 10.0    |
| Diphenyl-p-phenylenediamine | 1.0     |
| Tricresyl phosphate         | 3.0     |
| Mineral oil                 | 5.0     |
| Synthetic ester             | 71.0    |

With the exception of the sodium myristate, all of the materials employed in the preparation of this grease were the same as those employed in the grease of Example 1.

The grease was prepared in the following manner: A soap base was formed by saponifying a commercial myristic acid, having a saponification number of 250 and a titer, ° C. of 42.6, with the theoretical amount of sodium hydroxide in the presence of the mineral lubricating oil included in the grease, and then dehydrating for 1½ hours at 300-320° F. The dry indigo powder was then added to the concentrated soap solution and the temperature maintained at 300-320° F. for 1 hour longer with continuous stirring. The synthetic ester was then added gradually while the grease mixture was cooled down to 220° F. Near the end of the ester addition the inhibitors were added.

A short fiber blue grease was obtained having a dropping point of 402° F., and an ASTM worked penetration at 77° F. of 236.

In a number of other preparations of greases of the above type which were carried out employing the 1:1 indigo-sodium myristate mixture, the amount of thick-

ening agent required was from about 15 percent for a No. 1 grade grease up to about 20 percent for a No. 3 grade grease, as in Example 2. In comparison with these yields, a grease having an ASTM worked penetration at 77° F. of 274 (No. 2 grade) was obtained from 18.4 percent of sodium myristate in a typical preparation employing sodium myristate as the sole thickening agent. Mixtures of indigo and sodium myristate in proportions as high as 1:1 by weight are thus fully equivalent to sodium myristate alone in thickening power in these greases, the effectiveness of indigo as a thickening agent in combination with sodium myristate being in marked contrast to its deficiency in thickening power when employed as the sole thickening agent, as shown by Example 1. The use of higher proportions of indigo in the mixtures results in decreased yields, although proportions as high as 2:1 may be employed without decreasing the yields excessively. For example, a grease having an ASTM worked penetration at 77° F. of 373 (No. 0 grade) was prepared from 22.5 percent of a 2:1 indigo-sodium myristate mixture.

## EXAMPLE 3

A grease was prepared having the following composition by weight:

|                             | Percent |
|-----------------------------|---------|
| Indigo                      | 9.2     |
| Lithium myristate           | 8.6     |
| Diphenyl-p-phenylenediamine | 0.9     |
| Tricresyl phosphate         | 2.7     |
| Free alkali (as LiOH)       | 0.1     |
| Mineral oil                 | 8.5     |
| Synthetic ester             | 70.0    |

With the exception of the lithium myristate, all of the materials employed in the preparation of this grease were the same as those described in Example 1.

A grease was prepared substantially as described in Example 2, employing a commercial myristic acid of the same grade and saponifying in the presence of the mineral lubricating oil included in the grease, except that lithium hydroxide was employed in the saponification in place of sodium hydroxide, with a slight excess of lithium hydroxide over the amount theoretically required. Following the saponification the mixture was heated to 425° F. and cooled immediately to 300° F. The indigo was then added and the temperature maintained at 300° F. for 1 hour longer with continuous stirring. The addition of the synthetic ester and of the inhibitors was then carried out as described in Example 1. The product was finished by circulating it for 15 minutes in a Manton Gaulin Homogenizer at 4000 and 5000 pounds pressure.

A soft smooth blue grease was obtained having a dropping point of 462° F. and an ASTM worked penetration at 77° F. of 357.

## EXAMPLE 4

A grease was prepared having the following composition by weight:

|                             | Percent |
|-----------------------------|---------|
| Indigo                      | 10.0    |
| Sodium myristate            | 10.0    |
| Diphenyl-p-phenylenediamine | 1.0     |
| Tricresyl phosphate         | 3.0     |
| Mineral oil                 | 5.0     |
| Ditridecylazelate           | 71.0    |

All of the materials employed in the preparation of this grease were the same as those employed in the grease of Example 2, with the exception of the ditridecylazelate which was employed as the chief oleaginous component in place of the high molecular weight polyester of the foregoing examples.

The grease was prepared in the same manner described in Example 2.

A stiff blue grease was obtained having a dropping point of 388° F. and an ASTM worked penetration of 309.

Table I shows the high temperature performance properties of the greases of the above examples (greases Nos. 1, 2, 3 and 4, respectively), together with comparative data obtained upon a grease thickened with sodium myristate alone and upon greases containing carbon black as a thickening agent. The latter are included as representative of the other solid thickened greases of the prior art. These greases contained the same ester base and inhibitors as greases Nos. 1, 2 and 3, greases Nos. 5 and 7 containing 10 percent and 4 percent, respectively, of the mineral lubricating oil employed in the greases of the examples in admixture with the ester, and grease No. 6 containing the ester as the sole oleaginous component.

Table I  
HIGH TEMPERATURE PERFORMANCE TEST

| Grease No. | Thickener                              | Percent | Hours to Failure |          |
|------------|----------------------------------------|---------|------------------|----------|
|            |                                        |         | 350° F.          | 400° F.  |
| 1.....     | Indigo.....                            | 35.0    | 148              | -----    |
| 2.....     | 1:1 sodium myristate:indigo.....       | 20.0    | 1346             | 268      |
| 3.....     | 1:1 lithium myristate:indigo.....      | 17.8    | 894              | 131      |
| 4.....     | 1:1 sodium myristate:indigo.....       | 20.0    | 728              | 377; 273 |
| 5.....     | Sodium myristate.....                  | 18.4    | 191              | -----    |
| 6.....     | Carbon black.....                      | 15.0    | -----            | 217; 115 |
| 7.....     | 1:1 sodium myristate:carbon black..... | 15.0    | -----            | 121      |

The high temperature performance test of the foregoing table is a test for determining the performance characteristics of greases in anti-friction bearings at elevated temperatures and high rotative speeds. The test unit consists essentially of a steel spindle supported on ball bearings in an electrically heated housing and driven by an electric motor connected into an electric circuit containing a low amperage fuse 0.1 ampere below that required for full load running. The bearings are Normal-Hoffman ABEC No. 3 grade, and are mounted on a spindle approximately 5½ inches apart. A thrust load of 17.5 pounds is applied to the bearings. One bearing is used for test purposes and the second bearing, which is not heated, is used as a guide bearing. The test consists of operating the test bearing for twenty-four hours at 10,000 R. P. M. and at a temperature of from 250° F. to 450° F. followed by a shut down and cooling period of two hours, and repeating this cycle until the lubricant fails, which is indicated by rupture of the low amperage fuse in the motor circuit. In carrying out the test at 400° F. or above, Marlin Rockwell special heat treated high speed tool steel bearings with silver plated bronze retainers are used. In starting up the test, three grams of the test grease are charged to the test bearing and worked into and around the races and balls. The bearing is next rotated both clockwise and counterclockwise for one minute each at 200 R. P. M. and assembled into the test unit. The heaters and the motor are then started and the test bearing brought up to the test temperature as rapidly as possible, which requires 1.0 to 1.25 hours, while the spindle is rotated at a speed of 10,000 R. P. M. After 24 hours of operation the heaters and motors are shut off for 2 hours, during which the temperature of the test bearing drops to a minimum of 120-130° F. The total hours of operation, excluding the two hour shut-down periods, to the failure point is recorded as the "hours to failure."

As shown by the data given in Table I, greases containing both sodium or lithium myristate and indigo as thickening agents ran for several times as long in the high temperature performance test at 350° F. as did the greases thickened with either sodium myristate or indigo alone, showing that a pronounced synergistic effect is obtained upon the high temperature properties of a grease by the use of these two materials in combination as thickening agents. The unexpected nature of this effect is shown by the fact that the use of sodium myristate in

combination with carbon black only produced a grease which was inferior to the grease thickened with carbon black alone.

In addition to their very outstanding high temperature performance properties as discussed above, the greases prepared from indigo-soap mixtures in accordance with this invention had superior lubricating properties at low temperatures also, grease No. 2, for example, which is representative of a preferred embodiment of the invention, having appreciably lower low temperature torques at temperatures down to -60° F. than grease No. 5, wherein sodium myristate was employed as the sole thickening agent.

Obviously many modifications and variations of the invention, as hereinbefore set forth, may be made without departing from the spirit and scope thereof and therefore, only such limitations should be imposed as are indicated in the appended claims.

We claim:

1. A lubricating grease consisting essentially of an oleaginous liquid lubricating base thickened to a grease consistency with about 5 to 20 percent by weight based on the weight of the composition of indigo in finely divided form and about 5 to 20 percent by weight based on the weight of the composition of a soap selected from the group consisting of sodium and lithium soaps of fatty acids containing from 12 to 16 carbon atoms per molecule.
2. A lubricating grease according to claim 1 wherein the proportion of indigo to the said soap is from about 1:2 to about 2:1 by weight.
3. A lubricating grease according to claim 1 wherein the said soap is selected from the group consisting of sodium and lithium myristates.
4. A lubricating grease according to claim 1 wherein the said oleaginous liquid lubricating base comprises about 20-100 percent of a high molecular weight polyester of lubricating characteristics.
5. A lubricating grease according to claim 4 wherein the said polyester is a product obtained by reacting a dibasic aliphatic acid with a glycol and a compound selected from the group consisting of monohydric aliphatic alcohols and mono-carboxylic aliphatic acids.
6. A lubricating grease according to claim 4 wherein the said polyester is represented by the general formula
- 55 
$$R_2-OOC-R_1-COO-(R-OOC-R_1-COO)_x-R_2,$$
 wherein R is selected from the group consisting of aliphatic groups and aliphatic ether groups containing from 4 to 12 carbon atoms, R<sub>1</sub> is an aliphatic group containing from 1 to 12 carbon atoms, R<sub>2</sub> is an aliphatic group containing from 1 to 12 carbon atoms, and x is an integer from 1 to 5.
7. A lubricating grease according to claim 4 wherein the said polyester is represented by the general formula
- 55 
$$R_2-OOC-R_1-COO-(R-OOC-R_1-COO)_x-R_2,$$
 wherein R is an aliphatic group containing from 6 to 12 carbon atoms in branched chain arrangement, R<sub>1</sub> is an aliphatic group containing from 7 to 8 carbon atoms, R<sub>2</sub> is an aliphatic group containing from 4 to 9 carbon atoms in branched chain arrangement and x is an integer from 1 to 2.
8. A lubricating grease according to claim 4 wherein the said polyester is dodecylazelaate.
- 65 9. A lubricating grease consisting essentially of an oleaginous liquid lubricating base containing about 5-15 percent by weight of indigo in finely divided form, about 5-15 percent by weight of a soap selected from the group consisting of sodium and lithium myristates, about 0.1-8 percent of N,N' diphenyl para-phenylene diamine and about 0.3-15 percent by weight of tricresyl phosphate, said oleaginous liquid lubricating base comprising in minor proportion a mineral oil of lubricating characteristics and in major proportion a high molecular weight polyester of lubricating characteristics.

10. A lubricating grease according to claim 9 wherein the said polyester is represented by the general formula



wherein R is an aliphatic group containing from 4 to 12 carbon atoms, R<sub>1</sub> is an aliphatic group containing from 1 to 12 carbon atoms, R<sub>2</sub> is an aliphatic group containing from 1 to 12 carbon atoms, and x is an integer from 1 to 5.

11. A lubricating grease according to claim 10 wherein

the said polyester is a compound having the formula



12. A lubricating grease consisting essentially of an oleaginous liquid lubricating base containing about 5-15 percent by weight of indigo in finely divided form, about 5-15 percent by weight of sodium myristate, about 0.5-2

15

percent by weight of diphenyl-para-phenylene diamine and about 1-5 percent by weight of tricresyl phosphate, said oleaginous liquid lubricating base comprising in minor proportion a mineral oil of lubricating characteristics and in major proportion a polyester oil comprising essentially a compound of the formula



References Cited in the file of this patent

UNITED STATES PATENTS

|           |                 |               |
|-----------|-----------------|---------------|
| 2,542,570 | Puryear et al.  | Feb. 20, 1951 |
| 2,628,974 | Sanderson       | Feb. 17, 1953 |
| 2,639,266 | Dilworth et al. | May 19, 1953  |
| 2,663,690 | Eckert          | Dec. 22, 1953 |
| 2,663,691 | Dilworth        | Dec. 22, 1953 |
| 2,679,480 | Brannen et al.  | May 25, 1954  |